

## UNITED STATES PATENT OFFICE.

FREDERICK M. BECKET, OF NEW YORK, N. Y.

## ANODE FOR CHROMIUM PLATING.

No Drawing.

Application filed October 14, 1926. Serial No. 141,677.

This invention relates to the art of electroplating with metallic chromium, and comprises a soluble, chromium-containing cast anode for use in that operation.

5 Heretofore such anodes have commonly been made of cast chromium of the highest purity which was commercially available, hereafter for brevity designated "pure chromium".

10 Anodes of pure cast chromium present a number of undesirable properties. Pure chromium is quite viscous even when heated to a temperature well above its melting point, so that anodes can be cast from it only 15 in the simplest shapes. Such anodes are porous in varying degree, so that their rate of solution in the chromic acid electrolyte is irregular and impossible to predetermine. Furthermore, the crystal structure is such as

20 to affect most unfavorably the manner in which the anodes dissolve: instead of dissolving smoothly and regularly they tend to disintegrate, pieces of various sizes spalling or sloughing off and collecting at the bottom of the electrolytic cell, this involving 25 not only an increase in anode consumption but interfering with the operation of the cell.

These and perhaps other deficiencies of 30 cast chromium anodes have been heretofore recognized, and have been summarized somewhat inaccurately by characterizing such anodes as "brittle". It has been proposed to lessen this "brittleness" by additions of 35 lead, cobalt, iron or nickel; and while some of these additions in some proportions may diminish the so-called brittleness of the anode, they have the disadvantage that eventually they either foul the bath or have an 40 undesirable effect upon the quality of the deposit.

I have found that the defects mentioned above can be overcome by incorporating in the metal a controlled proportion of carbon, 45 the percentage being however materially below that which characterizes the known carbide  $\text{Cr}_3\text{C}_2$ , or which is present in the product resulting from the direct reduction of chromic acid by carbon in the electric furnace. Proportions of carbon as low as 0.5% 50 by weight exert a favorable effect, and proportions as high as 7.0% may be used. The advantages of the invention are attained in highest measure when the carbon content is

between 1 and 4 percent. As more fully explained hereinafter it is likewise of advantage to introduce silicon into the composition, in proportion depending on the particular results desired. In small proportion, say 1 to 2 percent in case of metal containing 1-4 percent of carbon, silicon increases 55 the fluidity of the molten metal and improves the crystalline structure of the cast article.

Anodes composed as above are much superior to anodes of pure cast chromium. They are less brittle, and there is much less breakage by handling both before and after they are placed in the bath. They have a better crystal structure or grain, which overcomes in large degree the difficulties of spalling and sloughing. The composition in molten state is much more fluid than pure chromium, and its melting point is lower; so that anodes can be successively cast of 75 almost any size or shape, which is a decided advantage in the many cases where it is desired to have the anode conform more or less to the shape of the cathode. Further, anodes of the above composition can be made 80 at a decidedly lower cost per unit of metallic chromium, as compared with anodes of pure cast chromium.

The electrolyte commonly and preferably used consists preponderantly of chromic acid 85 in aqueous solution. Since chromic acid oxidizes carbon quite readily, undergoing reduction to the trivalent state, and since trivalent chromium in large proportions is known to interfere with the proper course of 90 the electrolysis, it might naturally be assumed that carbon in any substantial proportion would be an objectional constituent of a chromium anode. I have found that this is in fact the case when the proportion of 95 carbon is substantially greater than seven percent; but proportions up to about seven percent may be successively used. As already stated my preferred proportions lie between one and four percent; but my invention is not limited to this last-mentioned range. Nor is it limited to the presence of 100 silicon, mentioned above as a desirable addition.

Silicon performs three distinct functions: 105  
1. In the smaller percentages it increases the fluidity of the molten metal, facilitates the casting, and improves the grain of the

cast article. These effects are already noticeable with silicon additions as low as 0.25 percent; but in case these are the chief objectives I prefer to introduce one to two percent of silicon, as already stated.

5 2. It is characteristic of metallic chromium anodes, used in a chromic acid electrolyte, that they tend to dissolve more rapidly than corresponds to the deposition of metal at the cathode, with the result that the concentration of the bath tends to increase progressively, and corresponding irregularities are introduced into the operation. This difficulty has been overcome in 10 the past by the simultaneous employment of soluble (chromium) and insoluble (lead) anodes, as disclosed in U. S. Patent 1,544,451 to Hambuechen. I have discovered that silicon, alloyed with the chromium in sufficient 15 proportions, say above 5 or 10 percent, reduces the rate of solution of the chromium in the electrolyte, such as aqueous solutions of chromic acid. The rate of solution of the chromium diminishes progressively although 20 not proportionately as the percentage of silicon is increased, until at about 40 percent silicon and upward, the balance almost all chromium, the alloy functions practically like an insoluble anode. Accordingly it is 25 possible, by properly adjusting the silicon content so to control the rate of solution of chromium as to obtain the desired balance 30 between the amount of metal dissolving at the anode and the amount deposited at the cathode, whereby the electrolyte remains 35 within the limits of concentration suitable for efficient plating. It is of course impossible to specify a definite silicon content which will accomplish this result in every 40 case, because the cathode efficiency varies considerably with the type of electrolyte used, its concentration and temperature, the current density, and other factors; but for use in baths consisting predominantly of 45 chromic acid in aqueous solution, I find that the optimum percentages of silicon lie between 10 and 35 percent; and in most cases between 20 and 30 percent.

3. Silicon in the higher ranges, say upward of about 10 percent, acts to exclude carbon from the resulting alloy, its effect increasing with increasing silicon content until practically carbon-free alloys are obtained when the silicon content is upward 55 of about 40 percent. Accordingly it is possible, by regulating the silicon content, to control the carbon content. Direct reduction of chromic acid by carbon in the electric furnace will yield a product containing 60 around 11 to 13 percent of carbon which as stated above is excessive for use in electroplating; whereas by adding to the charge sufficient silica to provide after reduction 65 10-15 percent of silicon in the alloy, or upward, the carbon content of the product may

be brought to any desired point within the permissible limits of 0.5-7 percent. At the same time the rate of anodic solution of chromium is lessened, and the rate at which the concentration of the electrolyte increases 70 is correspondingly lessened.

Having regard to all three of the above-described functions of silicon, as well as to the functions performed by carbon either in presence or absence of silicon, it will be understood that my present invention comprises broadly an anode of cast chromium metal containing about 0.5 to 7.0 percent of carbon, with or without silicon, the preferred carbon range being about 1 to 4 percent. 75 The invention comprises also a cast chromium anode containing carbon as above, and in addition thereto silicon in proportion between about 0.25 percent and 35.0 percent according to the particular objectives to be 80 attained. When the silicon is at or near the maximum mentioned the carbon will of course be at or near the minimum, by reason of the effect of silicon in excluding carbon 85 from these alloys.

90 I do not claim herein a substantially carbon-free chromium anode containing from about 0.25 to 35 percent of silicon, that subject matter being claimed in a copending application, Ser. No. 141,678, filed Oct. 14, 95 1926.

I claim:

1. A cast anode comprising chromium and about 0.5 to 7 percent of carbon.
2. A cast anode comprising chromium, silicon, and about 0.5 to 7 percent of carbon.
3. A cast anode comprising about 0.25 to 35.0 percent of silicon, about 0.5 to 7 percent of carbon, the balance substantially all chromium.
4. A cast anode comprising chromium and about 1 to 4 percent of carbon.
5. A cast anode comprising chromium, silicon, and about 1 to 4 percent of carbon.
6. In combination, an electrolyte consisting predominantly of an aqueous solution of chromic acid, and an anode comprising chromium, and about 0.5 to 7 percent of carbon.
7. In combination, an electrolyte consisting predominantly of an aqueous solution of chromic acid, and an anode comprising chromium, silicon, and about 0.5 to 7 percent of carbon.
8. In combination, an electrolyte consisting predominantly of an aqueous solution of chromic acid, and an anode comprising chromium, and carbon, substantially as described.
9. In combination, an electrolyte consisting predominantly of an aqueous solution of chromic acid, and an anode comprising chromium, carbon and silicon, substantially as described.

In testimony whereof, I affix my signature.  
FREDERICK M. BECKET.